# EUROPEAN PATENT SPECIFICATION

(11) **EP 0 117 328 B1**
(45) Date of publication and mention of the grant of the patent: **29.04.1987**
(21) Application number: 83301021.8
(22) Date of filing: 25.02.1983
(51) Int. Cl.: C10L 1/18, C10L 1/02

(54) **Liquid fuels containing corrosion inhibitors, and inhibitor concentrates**
Korrosionsinhibitoren enthaltende flüssige Brennstoffe, und Konzentrate von Inhibitoren
Combustibles liquides contenant des inhibiteurs de corrosion, et concentrés d'inhibiteurs

(43) Date of publication of application: 05.09.1984
(73) Proprietor: ETHYL PETROLEUM ADDITIVES LIMITED, Bracknell, Berkshire RG12 2UW (GB)
(72) Inventor: Burrows, Aubrey Lincoln, Bracknell, Berks. (GB); Field, Steven John, Wokingham, Berks. RG11 4UQ (GB); Brown, Alan, Bracknell, Berks. RG12 3TN (GB)
(74) Representative: Bizley, Richard Edward

## Description

In the past metal corrosion caused by conventional motor fuels such as gasoline was not much of a problem because such hydrocarbon fuels are inherently non-corrosive. However, with the advent of fuels containing alcohols such as gasohol or straight alcohol fuels, corrosion has become a major problem because such fuels are corrosive. It has been reported that this corrosion is due to the presence of acidic contaminants in such fuels such as formic acid. It is almost impossible to avoid such contaminants because they occur in fuel grade alcohols and are also formed in storage as normal alcohol oxidation products.

It is known from U.S. 4,305,730 that polymerized linoleic acid, especially trimer, is an effective corrosion inhibitor for alcohol-type motor fuels. It has now been discovered that the corrosion inhibiting properties of such polymerized polyunsaturated aliphatic monocarboxylic acids are improved by use of the co-additives described herein.

The use of an additive combination comprising a compound selected from the group consisting of dimers and trimers of ethylenic fatty acid (Cₗg--C₂₂ and a phenolic compound, preferably phenol itself, has been suggested in US 3,346,355 in relation to jet fuels. Such fuels contain 100% hydrocarbon mineral oil, usually a kerosene or naptha, and the additive serves as a lubricant and as an emulsification inhibitor. However, US 3,346,355 does not address itself to the problem of a fuel containing alcohol. As is explained further on, such fuels tend to corrode engine parts due to water content, and therefore there has been a need for an additive which will reduce such corrosion. A further problem arises in that certain additives tested actually tend to increase corrosion in some metals, whilst leaving others unaffected. An additive which on average over a range of likely contact metals gives good corrosion protection has therefore been sought.

According to the present invention metal corrosion caused by alcohol-type motor fuels is inhibited by adding to the fuel a combination of (A) polymerized polyunsaturated aliphatic monocarboxylic acid and (B) a sterically hindered phenol.

The invention provides a liquid fuel adapted for use in an internal combustion engine, the said fuel including a corrosion inhibiting amount of a combination of (A) a polymer of one or more C₁₆ to C₁₈ polyunsaturated aliphatic monocarboxylic acids and (B) at least one sterically hindered phenol, and the balance of the fuel comprising from 5 to 100 weight percent of one or more alcohols and 0 to 95 weight percent gasoline.

The additive combination of this invention can be beneficial in any engine fuel containing or consisting of an oxygenate. Such fuels include gasoline-alcohol mixtures referred to as "gasohol" as well as straight alcohol fuels. Useful alcohols are methanol, ethanol, n-propanol, isopropanol, isobutanol and the like. Gasohols usually contain about 2 to 30 volume percent alcohol. The most prevalent alcohols are methanol and ethanol. At concentrations above 10 volume percent phase separation problems are encountered especially in the presence of water. Phase separation can be minimised by including co-solvents in the gasohol such as ethers, ketones, esters and the like. An especially useful co-solvent is methyl tert-butyl ether which also serves to increase octane value.

The additive combination may be used at a concentration which provides the required amount of corrosion protection. A useful range is about 1 to 5000 parts per million (ppm). A more preferred range is about 5 to 2000 ppm and the most preferred concentration is 10 to 500 ppm.

Component A is a polymer of one or more 16 to 18 carbon polyunsaturated aliphatic monocarboxylic acids. Examples of these are linolenic acid and linolenic acid including mixtures thereof. The polymers comprise mainly dimers and trimers of the polyunsaturated acids. Suitable polymers of linolenic acid are available commercially. Mixtures high in trimer content are most preferred.

Component B of the combination is a hindered phenol. This includes any fuel (i.e. gasohol or alcohol fuels) soluble phenol having at least one bulky substituent ortho to a phenolic hydroxyl group.

Representative bulky substituents are secondary and tertiary alkyl (including cycloalkyl and alkyl (cycloalkyl) or aralkyl groups.

More preferably the hindered phenols are substituted in both positions ortho to a phenolic hydroxyl group with a secondary or tertiary alkyl or aralkyl group. Such phenols include
2,6-di-sec-butyl ph enol
2,6-diisopropyl phenol
2,6-di-tert-butylphenol
2,6-di-sec-octyl phenol
2-tert-butyl-6-(a-methylbenzyl)phenol
2-isopropyl-6-(a,a-dimethylbenzyl)phenol
2,6-di-(a-methylbenzyl)phenol
2,6-di-(a,a-dimethylbenzyl)phenol and the like.

In a highly preferred embodiment the hindered phenols are also substituted in the para position with an alkyl group containing 1 to about 20 carbon atoms. Examples of these hindered phenols are
2,6-di-tert-butyl-4-methyl phenol
2,6-di-tert-butyl-4-ethyl phenol
2,6-di-tert-butyl-4-(n-butyl) phenol
2,4,6-tri-tert-butyl phenol
2,6-di-tert-butyl-4-(sec-octyl) phenol
2,6-di-tert-butyl-4-(sec-eicosyl) phenol
2,6-diisopropyl-4-methylphenol
2,4,6-tri-sec-butyl phenol and the like.

In a still more preferred embodiment the hindered phenol is a 2,6-di-(a-methylbenzyl)-4-C₁-₂ₒ alkyl phenol. These include
2,6-di-(a-methylbenzyl)-4-methyl phenol
2,6-di-(a-methylbenzyl)-4-ethyl phenol
2,6-di-(a-methylbenzyl)-4-tert-butyl phenol
2,6-di-(a-methylbenzyl)-4-(n-butyl) phenol
2,6-di-(a-methylbenzyl)-4-(sec-octyl) phenol
2,6-di-(a-methylbenzyl)-4-nonylphenol
2,6-di-(a-methylbenzyl)-4-dodecylphenol
2,6-di-(a-methylbenzyl)-4-octadecylphenol
2,6-di-(a-methylbenzyl)^{;}4-eicosylphenol and the like.

Sterically hindered methylenebis phenols are also useful. These include 2,2' methylenebis-(4-alkyl-6-tert-alkyl phenols) and 4,4' methylenebis (2-alkyl-6-tert-alkyl phenols).

Representative examples of these are 2,2-methylenebis (4-methyl-6-tert-butyl phenol), 2,2' methylenebis-(4,6-di-tert-butyl phenol), 4,4' methylenebis (2,6-di-tert-butyl phenol), 4,4'-methylenebis-(2-methyl-6-tert-butyl phenol) and the like including mixtures thereof.

The most preferred hindered phenol is 2,6-di-(a-methylbenzyl)-4-nonylphenol. The nonyl group is readily available by alkylation with propylene trimer.

The weight ratio of component A to component B in the combination can vary over a wide range such as 1 to 10 parts A to 1 to 10 parts B. In a more preferred embodiment the weight ratio is about 0.5-5 parts component A for each part component B. In a still more preferred embodiment there are 0.6―4.0 parts component A per each part component B. The most preferred ratio is 1:1.

Components A and B can be separately added to the fuel. More preferably components A and B are pre-mixed to form a package and this package is added to the fuel in an amount sufficient to provide the required degree of corrosion protection.

Most preferably components A and B are also pre-mixed with a solvent to make handling and blending easier. Suitable solvents include alcohols (e.g. methanol, ethanol, isopropanol) ketones (acetone, methyl ethyl ketone) esters (tert-butyl acetate) and ethers (e.g. methyl tert-butyl ether).

Aromatic hydrocarbons are very useful solvents. These include benzene, toluene, xylene and the like. Excellent results have been obtained using xylene.

The concentration of the active components A and B in the package can vary widely. For example the active content can range from about 5 weight percent up to the solubility limit of A or B in the solvent. With xylene a total active content of about 5-25 weight percent is generally used, especially about 10 weight percent.

Tests were conducted to measure the anti-corrosion properties of the additive combination. In the test the corrosion of metal coupons immersed in test fluid was measured under different test conditions. Aluminium, brass, zinc, lead and copper coupons were used. the coupons were first cleaned with carborundum 40,^{*} washed with petroleum ether and oven dried for 10 minutes at 40°C.

Each coupon was weighed and then immersed in 130g of the test fluid in a sealed bottle for the specified time at the specified temperature.

At the end of the test period, the coupons were removed from the fuel; after loose deposits were removed with a light brush, the coupons were washed and dried as at the start of the test and then reweighed. Any change in coupon weight was recorded. Both gain and loss of weight indicate corrosion.

The corrosion was characterised by two modes, either weight loss by loss of metal or weight gain due to deposition of corrosion products, in the tests carried out below, visual examination of the coupons after test indicated that the two modes were mutually exclusive.

The first series of tests was conducted in various alcohol type fuels containing 100 ppm of the equal weight combination of linoleic acid polymer (mainly trimer) and 2,6-di-(α-methylbenzyl)-4-nonylphenol.

In this test series the temperature was ambient and immersion time 6 weeks. Results are given in the following table in terms of mg weight gain or loss. The value in parenthesis is the result without any inhibitor.

^{*}Silicon carbide powder which passes through a 40 mesh sieve.

In the next test series the coupons were placed in a bottle containing methanol doped with 100 ppm formic acid and 10 ppm methyl formate to increase test severity. The test additives were equal weight mixture of linoleic acid trimer and various hindered phenols as shown in Table II. Additive concentration was 100 ppm. The bottles with the test coupons were stored two weeks at 40°C. Weight change due to corrosion is shown in Table II.

Further tests were conducted which show the synergistic results obtained with this combination of additives. These tests were in methanol doped with 100 ppm formic acid and 10 ppm methyl formate. The metal coupons were immersed in the fuel and stored two weeks at 40°C.

Additive D was 2,6-di-(a-methylbenzyl)-4-nonylphenol. Additive E was linoleic acid trimer. Additive D+E was an equal weight mixture of D and E. Total inhibitor concentration in each test was 300 ppm.

These results show that the combination gives better results than would be expected from the results obtained with each component.

In the next test series the fuel was methanol doped with 100 ppm formic acid and 10 ppm methyl formate. The metal coupons were only partially immersed (approx 50%) and the bottles were stored two weeks at 40°C. The additive was a 50/50 mixture of linoleic acid trimer and 2,6-di-(a-methylbenzyl)-4-nonylphenol. Additive concentration was 300 ppm in each samples. Test results are given in Table IV.

The next test was again conducted in gasohol containing 15 vol percent methanol and doped with 100 ppm formic acid and 10 ppm methyl formate. The metal coupons were fully immersed and stored two weeks at 40°C. Additive concentration was 100 ppm. Table V gives the test results with and without the test additive. The test additive was an equal weight mixture of linoleic acid trimer and various hindered phenols as indicated.

The test results show that while not equally effective on all metals in all fuels, the additive combination on average gives very good corrosion protection.

## Claims

1. A liquid fuel adapted for use in an internal combustion engine, the said fuel including a corrosion inhibiting amount of a combination of (A) a polymer of one or more C₁₆ to C₁₈ polyunsaturated aliphatic monocarboxylic acids and (B) at least one sterically hindered phenol and the balance of the fuel comprising from 5 to 100 weight percent of one or more alcohols and 0 to 95 weight percent gasoline.

2. A liquid fuel as claimed in claim 1 wherein said polymer of one or more C₁₆ to C₁₈ polyunsaturated aliphatic monocarboxylic acids comprises mainly linoleic acid dimer, trimer or mixtures thereof.

3. A liquid fuel as claimed in claim 1 or claim 2 wherein the or each said hindered phenol is substituted in both positions ortho to the phenolic hydroxyl group with a secondary or tertiary alkyl or aralkyl group.

4. A liquid fuel as claimed in claim 3 wherein said phenol is a 2,6-di-(α-methylbenzyl)-4-C₁₋₂₀-alkylphenol.

5. A liquid fuel as claimed in claim 4 wherein said phenol is 2,6-di-(a-methyl-benzyl)-4-nonylphenol.

6. A liquid fuel as claimed in claim 3 wherein said phenol is a 2,6-di-tert-butyl-4-C1-2o alkyl phenol.

7. A liquid fuel as claimed in claim 6 wherein said phenol is 2,6-di-tert-butyl-4-butylphenol.

8. A liquid fuel as claimed in claim 6 wherein said phenol is 2,6-di-tert-butyl-4-methylphenol.

9. A liquid fuel as claimed in claim 3 wherein said phenol is 4,4'-methylenebis-2,6-di-tert-butylphenol.

10. A liquid fuel as claimed in claim 3 wherein said phenol is 2,6-di-tert-butylphenol.

11. A corrosion inhibitor concentrate comprising a solvent containing at least 5% by weight of a combination of (A) a polymer of one or more C₁₆ to C₁₈ polyunsaturated aliphatic monocarboxylic acids and (B) at least one sterically hindered phenol.

## Patentansprüche

1. Kraftstoff zur Verwendung in einem Verbrennungsmotor, wobei der Kraftstoff eine korrosionsinhibierende Menge einer Kombination aus (A) einem Polymer aus einer oder mererer C₁₆ bis C₁₈ polyungesättigter aliphatischer Monocarbonsäuren und (B) mindestens einem sterisch gehinderten Phenol enthält und der Rest des Kraftstoffs 5 bis 1-00 Gew.-% eines oder mehrerer Alkohole sowie 0 bis.95 Gew.-% Benzin enthält.

2. Kraftstoff nach Anspruch 1, worin das Polymer aus einer oder mehreren C,₆ bis C₁₈ polyungesättigten aliphatischen Monocarbonsäuren, hauptsächlich Linolsäuredimer, -trimer oder ihrer Gemische enthält.

3. Kraftstoff nach Anspruch 1 oder 2, worin das oder jedes gehinderte Phenol in beiden Orthostellungen zur phenolischen Hydroxylgruppe mit einer sekundären oder tertiären Alkyl- oder Aralkylgruppe substituiert ist.

4. Kraftstoff nach Anspruch 3, worin das Phenol 2,6-di-(a-methylbenzyl)-4-C₁-₂ₒ-alkylphenol ist.

5. Kraftstoff nach Anspruch 4, worin das Phenol 2,6-di-(α-methylbenzyl)-4-nonylphenol ist.

6. Kraftstoff nach Anspruch 3, worin das Phenol 2,6-di-tert-butyl-4-C₁₋₂₀-alkylphenol ist.

7. Kraftstoff nach Anspruch 6, worin das Phenol 2,6-di-tert-butyl-4-butylphenol ist.

8. Kraftstoff nach Anspruch 6, worin das Phenol 2,6-di-tert-butyl-4-methylphenol ist.

9. Kraftstoff nach Anspruch 3, worin das Phenol 4,4'-methylenbis-2,6-di-tert-butylphenol ist.

10. Kraftstoff nach Anspruch 3, worin das Phenol 2,6-di-tert-butylphenol ist.

11. Korrosionsinhibitorkonzentrat enthaltend ein Lösungsmittel, das mindestens 5 Gew.-% einer Kombination aus (A) einem Polymer einer oder mehrerer C,₆ bis C₁₈ polyungesättigter aliphatischer Monocarbonsäuren und (B) mindestens ein sterisch gehindertes Phenol enthält.

## Revendications

1. Carburant liquide destiné à être utilisé dans un moteur à combustion interne, ledit carburant comprenant une quantité inhibitrice de corrosion d'une association de (A) un polymère formé à partir de un ou plusieurs acides monocarboxyliques aliphatiques polyinsaturés en C₁₆ à C₁₈ et (B) au moins un phénol à encombrement stérique, le reste du carburant comprenant 5 à 100% en poids d'un ou plusieurs alcools et 0 à 95% en poids d'essence.

2. Carburant liquide suivant la revendication 1, dans lequel ledit polymère formé à partir d'un ou plusieurs acides monocarboxyliques aliphatiques polyinsaturés en C₁₆ à C₁₈ comprend principalement un dimère d'acide linoléique, un trimère d'acide linoléique ou leurs mélanges.

3. Carburant liquid suivant la revendication 1 ou 2, dans lequel le phénol à encombrement stérique, ou chacun desdits phénols, est substitué dans les deux positions ortho par rapport au groupe hydroxyle phénolique avec un groupe alkyle ou aralkyle secondaire ou tertiaire.

4. Carburant liquide suivant la revendication 3, dans lequel ledit phénol est un 2,6-di-(a-méthyl- benzyl)-4-(alkyl en C₁―C₂₀)phénol.

5. Carburant liquide suivant la revendication 4, dans lequel ledit phénol est le 2,6-di-(a-méthyl- benzyl)-4-nonylphénol.

6. Carburant liquide suivant la revendication 3, dans lequel ledit phénol est un 2,6-di-tertiobutyl-4-(alkyl en C₁―C₂₀)phénol.

7. Carburant liquide suivant la revendication 6, dans lequel ledit phénol est le 2,6-di-tertio-butyl-4-butylphénol.

8. Carburant liquide suivant la revendication 6, dans lequel ledit phénol est le 2,6-di-tertio-butyl-4-méthylphénol.

9. Carburant liquide suivant la revendication 3, dans lequel ledit phénol est le 4,4'-méthylène-bis-2,6-di-tertio-butylphénol.

10. Carburant liquide suivant la revendication 3, dans lequel ledit phénol est le 2,6-di-tertio-butyl- phénol.

11. Concentré inhibiteur de corrosion comprenant un solvant contenant au moins 5% en poids d'une association de (A) un polymère formé à partir d'un ou plusieurs acides monocarboxyliques aliphatiques .polyinsaturés en C₁₆ à C₁₈ et (B) au moins un phénol à encombrement stérique.
